

Jan. 1, 1924

1,479,121

W. H. WASHBURN

TWO-PIECE VALVE AND METHOD OF MAKING SAME

Filed Oct. 24, 1921



## UNITED STATES PATENT OFFICE.

WILLIAM H. WASHBURN, OF CHICAGO, ILLINOIS, ASSIGNOR TO THE OLIVER TYPE-WRITER COMPANY, OF CHICAGO, ILLINOIS, A CORPORATION OF ILLINOIS.

## TWO-PIECE VALVE AND METHOD OF MAKING SAME

Application filed October 24, 1921. Serial No. 509,948.

*To all whom it may concern:*

Be it known that I, WILLIAM H. WASHBURN, a citizen of the United States, residing at Chicago, county of Cook, State of Illinois, have invented a certain new and useful Improvement in Two-Piece Valves and Methods of Making Same, and declare the following to be a full, clear, and exact description of the same, such as will enable others skilled in the art to which it pertains to make and use the same, reference being had to the accompanying drawings, which form a part of this specification.

It is desirable in poppet valves for internal combustion engines to have the head made out of a heat-resisting alloy while the stem is made out of a wear-resisting or friction-resisting alloy. Heretofore the common practice of making valves of this kind has been to screw the heads on the ends of the stems and, after riveting over the ends of the stems somewhat, welding the heads and stems together. This is not only an expensive process but it introduces welding stresses which frequently cause warping in the stems just under the heads or close to the points where the welds are made. Consequently valves made in the manner just described are not only expensive but they are frequently defective.

The object of the present invention is to produce a perfect two-part poppet valve in a simple and novel way and at a low manufacturing cost.

The various features of novelty whereby my invention is characterized will herein-after be pointed out with particularity in the claims; but, for a full understanding of my invention and of its object and advantages, reference may be had to the following detailed description taken in connection with the accompanying drawing, wherein:

Figure 1 is a vertical section through a pair of forming dies ready to close upon a rudimentary valve head and fashion it and secure it to a stem held in position to receive it;

Fig. 2 is a view similar to Fig. 1 showing the condition existing when the dies have been closed on the work; and

Fig. 3 is a side elevation of the completed valve head and the adjacent portion of the stem.

In accordance with my invention I first make a finished stem, something which can be accomplished at a very low cost by automatic machinery into which is fed rod or heavy wire stock. A rudimentary head is then placed on the end of a stem and is simultaneously forged into a completed head and attached to the stem in such a manner that no stresses tending to produce warping or distortion are produced, and permitting the completed valve to be placed directly in service after the single finishing operation of grinding the valve face.

Referring to the drawing, 1 represents the lower die and 2 the upper die of a forging machine. The lower die has a central hole or chamber 3 into which a valve stem 4 accurately fits. The hole or chamber is closed at the bottom so that the valve stem will rest on a solid support at its lower end. In the top of the lower die, co-axial with the hole 3, is a mold cavity 5 having the shape of a completed valve-head. The bottom of the upper die may be simply a flat surface although there is preferably a central recess or depression 6 slightly larger in diameter than the diameter of the valve stem, so as to insure that there will always be a clearance between the upper end of the valve stem and the upper die or between the upper die and any metal which might flow across the top of the valve stem from the rudimentary valve during the forging operation.

That portion of the valve stem which lies within the mold cavity 5 when the stem is dropped into the lower die is provided with superficial irregularities adapted to interlock with the metal of the valve-head. These irregularities preferably take the form of an ordinary screw thread 7 extending throughout the length of that portion of the stem that lies above the bottom of the mold cavity.

While the valve stem is placed in the die in a finished condition, the head, when placed in the die, is a mere rudimentary blank in the form of a thick washer, as indicated at 8. The hole 9 in the blank is made somewhat larger in diameter than the diameter of the screw threaded portion of the stem and, instead of being cylindrical, is preferably made in the form of a frustum of a cone the smaller end of which lies at

the bottom when the blank is placed in the machine. The thinnest portions of valves of the kind under consideration are the marginal portions and there is usually a gradual increase in thickness toward the center so that the thickness or depth is greatest at the center. I therefore prefer to make the valve-head blank thickest at the middle and decreasing gradually in thickness toward the periphery.

In building a valve, a stem is dropped down into the lower die, the stem being at ordinary room temperature. The blank for the head is heated to a high temperature, preferably one approaching welding heat. The hot blank is then dropped into the mold cavity in the lower die and the upper die is driven down. The shape of the blank is such that in the first instance it is supported only at the margin, so that as soon as the upper die engages with the top of the blank it starts to press the center of the blank down. Since the opening in the blank is larger in diameter than the stem, the downward movement of the center of the blank takes place just as though the stem were not present. Only after the bottom of the blank has been shaped to the mold cavity excepting only at the middle where the boss or hub in the completed valve is to appear, the continued downward movement of the upper die forces the metal of the blank in the vicinity of the stem downwardly and also inwardly toward the axis of the stem. As the metal flows down into the bottom portion 10 of the mold cavity which is for the purpose of giving shape to the hub or boss on the under side of the valve-head, it finds itself confined by a rigid surrounding wall and it therefore can flow only inwardly toward the axis of the valve, namely upon the screw threads. The definite movement of the metal in the head toward the axis begins at the bottom and progresses toward the top so that it may be said that the head is forged or molded so as to bring it progressively into interlocking engagement with the screw threads on the stem from the bottom of the head toward the top. This is considered of importance because the advantages secured from the working of the metal of the head in forging it into shape are not lost through the creation of shearing stresses which begin to shear away the metal of the head lying next to the valve stem while the downward flow or movement of the main portion of the metal is taking place. When the upper die is fully closed upon the lower die there will of course be a downward pressure on the metal of the head immediately adjacent to and surrounding the stem, but this will serve only to insure perfect contact at all times between the screw threads and the metal of the head, and there may also be a slight dis-

tortion of the lowermost screw threads which will produce a locking effect if it be attempted to unscrew the head.

It will be seen that the stem is not subjected to any forces which will affect it in any way, the principal stresses that are applied to the stem being the radial stresses as the material of the head is forged inwardly toward the axis. It will also be seen that by forging the head while heated to a degree which permits it to flow readily under pressure, there will be no unbalanced internal stresses which might produce warping or distortion after removal of the valve from the dies. Consequently when the valve is removed from the mold it is ready to be put into use as soon as it becomes cool, the only finishing operation that is necessary being the grinding of the valve face.

When the two parts of the valve are assembled in the press the difference in temperature between them is greater than it will ever be thereafter, the stem being practically cold, namely at room temperature, and the valve being at approximately a welding heat. At the end of the forging operation, (which of course takes only a fraction of a second,) the valve head is still very hot and, as it cools, it contracts both in the axial direction and in the radial direction, thus shrinking it tightly upon the stem and making it substantially integral with the stem. When the valve is put into use that part of the stem surrounded by the head becomes just as hot as the head itself, thereby maintaining the relative condition which existed when both the stem and the head were cold. In other words, when the head cools after the valve has been taken out of the dies, it shrinks and increases its grip on the comparatively cool stem, which grip would be decreased if the head could again be heated without correspondingly heating the stem, but which will remain practically constant if the stem be heated at the same time that the head is heated as is the case when the valve is put into service.

I claim:

1. The method of making a two-part valve which consists in inserting the screw threaded end of a stem into a cone-shaped hole in a valve-head blank larger in diameter at the smaller end than the stem, and then forging the blank so as to cause the metal to flow toward the center and progressively fill the screw threads in the stem beginning with the threads in the small end of the hole and simultaneously give to the blank the contour of a valve-head.

2. The method of making a two-part valve which consists in resting one end of a cold finished stem on a support, locating a heated washer-like blank of approximately the diameter of the valve head to be formed so that it surrounds the stem in the vicinity of

- the other end and leaves the latter end free and exposed, then forging the blank without imposing any forging pressure on the last mentioned end of the stem so as to cause the metal of the blank to flow into intimate contact with the stem and simultaneously give to the blank the shape of a valve head, and then completing the valve by grinding the valve face.
- 10 3. The method of making a two-part valve which consists in inserting a stem into a cone-shaped hole in a heated "valve-head" blank, and then forging the blank so as to cause the metal to flow towards the center and progressively engage the stem from the portion lying adjacent to the smaller end of the hole to that portion lying adjacent to the larger end of the hole and simultaneously give to the blank the contour of a valve head.
- 15 4. The method of making a two-part valve which consists in inserting the end of a stem having grooves extending around the same, into a cone-shaped hole in a hot valve-head blank larger in diameter at the smaller end than the stem, and then forging the blank so as to cause the metal to flow toward the center and progressively fill the grooves in the stem beginning with the groove in the small end of the hole and simultaneously give to the blank the contour of a valve head.
- 20 5. The method of making a two-part valve which consists in inserting a stem into a hole of larger diameter extending through a hot valve-head blank, so as to leave the end of the stem exposed and free, and then forging the blank so as to cause the metal to flow towards the center into intimate contact with the stem and simultaneously give to the blank the shape of a valve head, without exerting any forging pressure on the said end of the stem in the direction of the length of the stem.
- 25 6. The method of making a two-part valve which consists in inserting a comparatively cold stem into a hole of larger diameter extending through a highly heated valve-head blank, and then forging the blank to cause the metal to flow toward the center into intimate contact with the stem and simultaneously give to the blank the shape of a valve head without exerting any forging pressure on the stem in the direction of the length of the stem.
- 30 7. The method of making a two-part valve which consists in inserting a shouldered portion of a stem into a hole of larger diameter extending through a heated valve-head blank, and then forging the blank without exerting any forging pressure on the exposed end of the stem, so as to cause the metal to flow toward the center into intimate contact with the stem and simultaneously give to the blank the contour of a valve head.
- 35 8. The method of making a two-part valve which consists in inserting a shouldered portion of a cold stem into a hole of larger diameter extending through a highly heated valve-head blank so as to leave an end of the stem adjacent to the blank free and exposed, and then forging the blank by exerting a pressure on the same only on the surfaces thereof surrounding said hole and without exerting any forging pressure on said exposed end of the stem so as to cause the metal to flow toward the center into intimate contact with the stem and simultaneously give to the blank the contour of a valve head.
- 40 9. The method of making a two-part valve which consists in heating a washer-like blank of approximately the diameter of the valve head to be formed, inserting in the hole in the blank a transversely-shouldered part near one end of a stem smaller in diameter than said hole; and then applying pressure to the blank only, while the stem is left free, to cause the metal of the blank to flow toward the center into intimate contact with the stem and simultaneously give to the blank the shape of a valve head.
- 45 10. The method of making a two-part valve which consists in heating a washer-like blank of approximately the diameter of the valve head to be formed, inserting in the hole in the blank a part near one end of a stem smaller in diameter than said hole, and then forging the blank in dies one of which has a recess somewhat larger in diameter than the stem and adapted to register with said end of the stem when the dies are closed and thus avoid placing endwise forging pressure on the stem.
- 50 11. The method of making a two-part valve which consists in resting one end of a cold stem on a support, locating a heated washer-like blank of approximately the diameter of the valve head to be formed so that it surrounds the stem in the vicinity of the other end and leaves the latter end free and exposed, and then forging the blank without imposing any forging pressure on the last mentioned end of the stem so as to cause the metal of the blank to flow into intimate contact with the stem and simultaneously give to the blank the shape of a valve head.
- 55 In testimony whereof, I sign this specification.

WILLIAM H. WASHBURN.